

## UNITED STATES PATENT OFFICE

2,586,647

## ALUMINUM ALLOY

Harold Ernest Gresham, Little Eaton, and Douglas Wilson Hall, West Monkseaton, England, assignors to Rolls-Royce Limited, Derby, England

No Drawing. Application February 4, 1947, Serial No. 726,440. In Great Britain February 8, 1946

1 Claim. (Cl. 75—147)

1

It is well known that artificially aged aluminium alloys when subjected to severe corrosion conditions such as salt water, mist or spray, are very prone to intercrystalline attack.

In order to avoid this corrosion effect high strength aluminium alloys such as Duralumin are coated with pure aluminium to give such materials as "Alclad."

Alloys are also used of aluminium with up to 3.5 per cent of magnesium and sometimes small additions of manganese. These alloys are of low strength but have high resistance to corrosion. They are however not susceptible to artificial age hardening unless other elements are added, and the elements hitherto added for this purpose have destroyed the corrosion resisting properties of the alloy.

We have found that the addition of silver 0.2 to 2% to an aluminium alloy containing 1 to 3.5% magnesium gives an alloy which responds to artificial ageing, moreover this alloy is equal to or more resistant to corrosion than the plain magnesium aluminium alloy. As a result of this artificial ageing the alloy is also stronger than the plain alloy.

The alloy preferably contains manganese and is of the following composition:

|                         | Per cent    |
|-------------------------|-------------|
| Magnesium               | 1 to 3.5    |
| Silver                  | 0.20 to 2.0 |
| Manganese               | 0.05 to 1.0 |
| Aluminium the remainder |             |

Other elements can be present in limited amounts.

Silicon which is an impurity in aluminium should not exceed 0.35 per cent and is preferably kept as low as possible.

Nickel can be present up to 2.0 per cent. Iron, zinc, cobalt and zirconium may be present up to 1 per cent of each without seriously affecting the alloy.

Antimony, tin, chromium, may be present up to 0.5 per cent of each.

Copper, titanium, beryllium, vanadium, molybdenum, tungsten, niobium, cerium and the rare earth elements may be used as cleaners and grain refiners up to a total of 1 per cent but with not more than 0.3 per cent of any individual element. For the rare earths Misch metal may be used and may be present up to 1.0 per cent. Other elements such as lithium, cadmium, calcium, strontium, barium, thorium, arsenic, lead, bismuth and others may be tolerated up to 0.1 per cent individually and 0.3 per cent total.

2

The preferred heat treatment is to give solution heat treatment at 520° to 550° C. for 1 to 20 hours, to quench in water and age at 160° C. to 200° C. for 8 to 30 hours.

5 An alloy of the following composition:

|                         | Per cent |
|-------------------------|----------|
| Magnesium               | 2.5      |
| Silver                  | 0.5      |
| Manganese               | 0.15     |
| Silicon                 | 0.20     |
| Iron                    | 0.25     |
| Aluminium the remainder |          |

10 was hot forged, solution heat treated at 550° C. for 2½ hours quenched in water and aged for 24 hours at 165° C. It gave a tensile strength of 18.5 tons per square inch with 22 per cent elongation. The rise in Brinell hardness which occurred as a result of the artificial ageing was 40 points Brinell, i. e. it rose from 45 to 85 Brinell. Without the silver addition it would have remained at about 45 Brinell.

15 A well known widely used aluminium alloy containing 3.5 per cent magnesium, 0.5 per cent manganese, 0.25 per cent iron and 0.20 per cent silicon cast in the same mould and hot forged in the same manner was corrosion tested along with the new alloy.

20 The results before and after nine weeks intensive corrosion in sea water are as follows:

|                  | New Alloy        |             | Well-known Alloy |             |
|------------------|------------------|-------------|------------------|-------------|
|                  | Tensile Strength | Elong.      | Tensile Strength | Elong.      |
| 35               |                  |             |                  |             |
| Before Corrosion | Tons 18.5        | Per Cent 22 | Tons 17          | Per Cent 18 |
| After Corrosion  | 16.3             | 17          | 13               | 7.5         |

40 It will thus be seen that the new alloy is twice as resistant to corrosion as judged by loss of properties.

45 If zinc is added the initial strength is increased, but there is a slightly greater reduction of elongation after the corrosion test. An alloy similar in composition to the above example of the new alloy, but containing 0.4 per cent zinc gave the following figures after similar treatment:

|                  | Tensile Strength |          | Elongation |
|------------------|------------------|----------|------------|
|                  | Tons             | Per cent |            |
| 50               |                  |          |            |
| Before Corrosion | 19.2             | 20       |            |
| After Corrosion  | 17.0             | 12       |            |

It will be observed this alloy is also superior to the well known alloy.

The alloy can be used either as castings or as forgings, being heat treated in either case to suit requirements. With forgings cold work may be introduced as a means of strengthening the alloy and may be carried out either after solution heat treatment and before ageing, or after the full heat treatment.

This alloy is also good for welding.

What we claim is:

An age hardened aluminum base alloy resistant to severe corrosion conditions and comprising an aluminum base alloy consisting of 94.5-98.8% aluminum, 1-3.5% magnesium and 0.20-2.0% silver in the condition produced by solution heat treatment of 1-20 hours at 520-550° C., followed by quenching and 8-30 hours ageing at 160-200° C.

HAROLD ERNEST GRESHAM.  
DOUGLAS WILSON HALL.

#### REFERENCES CITED

The following references are of record in the file of this patent:

##### UNITED STATES PATENTS

| Number    | Name        | Date          |
|-----------|-------------|---------------|
| 1,920,090 | Lyon et al. | July 25, 1933 |
| 2,336,512 | Stroup      | Dec. 14, 1943 |
| 2,388,540 | Hartmann    | Nov. 6, 1945  |

##### FOREIGN PATENTS

| Number  | Country       | Date         |
|---------|---------------|--------------|
| 432,964 | Great Britain | Aug. 2, 1935 |
| 132,612 | Germany       | Apr. 5, 1901 |

##### OTHER REFERENCES

"Practical Metallurgy," published by the American Society for Metals, 1940, page 32.

"Age Hardening of Metals," published by the American Society for Metals, 1940, page 441.